

## UNITED STATES PATENT OFFICE

1,936,525

## PROCESS OF MANUFACTURING PHOTOSENSITIVE BODIES

Carl Roehrich, Berlin, Germany, assignor to the firm Silfree Aktiengesellschaft (Silfree Limited), Vaduz, Lichtenstein

No Drawing. Application January 9, 1929, Serial No. 331,384, and in Germany January 21, 1928

7 Claims. (Cl. 95—7)

The present invention concerns an improved method of manufacturing sensitive plates, films and the like.

It has been hitherto known to manufacture 5 sensitive plates, films and the like, by coating a support, consisting of glass, celluloid or any other transparent material or of thin metal foils, with a layer of colloids, such as gelatin, glues or the like, which is sensitized by impregnation with 10 suitable chemicals.

Various means and numerous methods of impregnating the plates and films are known. Silver-salts are very frequently used as sensitizing chemicals, the films, prepared with said salts, 15 on being exposed to the light, turning more or less dark at all parts which have been exposed to the light.

Other wellknown sensitizers cause the gelatin to harden by the action of the light at those 20 parts of the film, which had been exposed to the light, whilst the parts protected against the light are left soluble and absorbent. The present invention relates especially to plates, films and the like, sensitized in this way.

25 After the exposure, the film has to be subjected to a further treatment for the purpose of rendering the picture visible. This can be reached, for example, by the action of certain dyes or other sensitizers, which are absorbed by the non-hardened parts of gelatin, whilst the hardened parts are left free.

As sensitizers of this second type, chromic acid salts are generally used. The chromic acid salts are often applied to the plates or films together 35 with other metal salts in aqueous solution or in alcoholic solution diluted with water, the impregnation being frequently carried out by immersing the material to be sensitized in a bath of the said solutions. After absorption is completed the films are subjected to a subsequent 40 drying process and are then ready for use.

On removing the films from said sensitizing bath, traces of the sensitizing solution remain 45 on the surface of the film, besides those parts of the solution absorbed by the colloid layer.

Thorough investigations have shown that these remaining traces are not uniformly distributed over the surface of the film, but that they form 50 globules. Thus the surface looks like a fatty surface, on which water has been applied.

During the drying process, the liquid solvent is evaporated from the globules and sediments are formed on the surface of the film.

55 It was further found, that the higher the per-

centage of salts in the solution, used for the impregnation, the more sediment accrues.

The appearance of these sediments decreases considerably the usefulness of the plates or films. Firstly, the colloid-layer being non-uniformly sensitized, the light must act more weakly on the weaker sensitized parts of the layer than on the stronger sensitized ones, causing irregularities and shadows on the subsequently produced picture.

A further source of faults lies in the alterations effected on the entering light by means of the more or less crystallized sediments, inasmuch as this light is reflected, broken and diffracted by each single crystal face. It is therefore impossible for the entering light to penetrate such films uninterrupted, whereby the quality of the picture obtained is further impaired.

Furthermore these sediments are nearly always coloured, in most cases yellow, thereby acting as coloured filters for the incident light. This impairs the action of the light, as coloured filters are known to absorb parts of the light, which therefore can not act on the deeper layers of the colloid. The sediments thus cause 80 also considerable losses of light energy. The present invention has for its purpose to avoid the disadvantages mentioned above.

One object of the invention is to prepare sensitive plates, films and the like, the surfaces of 85 which are free from sediments.

Another feature of the invention is to manufacture sensitive material, sensitized by means of chrome salts, the sensitizers being uniformly distributed throughout the colloid layer.

A further feature is to provide such sensitized layers, into which the incident light may freely enter, uninterrupted by diffracting faces.

Still another feature of the present invention is to manufacture sensitive films and plates, the 95 surface of which is free from coloured sediments, thereby avoiding losses of energy of the incident light, effected by absorption in the coloured sediments.

From the foregoing can be seen that the pictures produced from such films or plates, free 100 from sediments, will be clearer, sharper and free from shadows, veils and other irregularities, and that these good results moreover can be attained by using for the exposure less light energy or— 105 which is a very considerable advantage in practical work—a shorter duration of exposure than hitherto.

It was first attempted to achieve this end by treating the films and the like with water, after 110

impregnation with the sensitizing solution, where it was found that no or only the very slightest decrease of sediment was effected by this treatment. Satisfactory results were, however, not reached by this method.

Further experiments showed that the treatment of the sensitive material with diluted alcohols gives very satisfactory results. For this purpose the sensitive films or plates, after impregnation with the sensitizing solution as above mentioned, are subjected to the action of an alcohol. This treatment may be performed in any suitable way, for example by running the sensitive material under treatment through weak alcoholic solution or by applying said solution to the sensitive surface of the material in any well-known way.

When thus treated, the globules on the surface of the film disappear, the remaining traces of liquid are uniformly distributed over the whole surface, and no sediments appear, when the film is dried.

This result may be considered as effected by loosening the surface tension by the alcohol, thereby balancing the forces acting from the surface of the film on the liquid.

A solution containing a 10% alcohol solution has been found sufficient for most purposes. Ethyl alcohol for example may be used, other alcohols however giving good results too. Precaution must be taken with regard to the duration of this treatment, as the aqueous solution naturally lixiviates the sensitized layer, and therefore may reduce the sensitiveness should the treatment be continued too long. It will suffice in most cases to submit the film to the alcohol for about 12 seconds. As a rule the duration of this treatment is only a fraction of the previous time of impregnation, and may range for example between 10 and 20 seconds.

The after-treatment described may be performed immediately after the sensitization is concluded or before the sensitizing solution has perfectly dried.

In the following a preferred form of this treatment is described as an example, without however limiting the invention to the particular details of the method, as given below.

A transparent film of celluloid is coated with a layer of gelatin, and is then, for the purpose of sensitizing, immersed in a bath containing:

|                       |           |
|-----------------------|-----------|
| Bichromate of ammonia | 80 gr.    |
| Sulfate of copper     | 1.5 gr.   |
| Ammonia               | 200 ccm.  |
| Alcohol               | 150 ccm.  |
| Water                 | 1000 ccm. |

After remaining in this bath for about 3 minutes, the film is removed and immediately transferred to a second bath containing 10% ethyl alcohol in water. After about 12 seconds, the film is removed and subsequently dried. The drying is preferably carried out in one of the well-known drying devices with warm air, a temperature of about 23-24° C. being suitable. For large scale manufacture the above proposed after-treatment may be combined with the usual continuous process of manufacturing films. This may be done for instance by guiding the film uninterruptedly and continuously through the second bath, after having been sensitized in the first bath, and by then drying the film uninterruptedly and continuously.

From this method a film results, the surface of which is free from sediments, and wherein the sensitizers are uniformly distributed. During the

exposure the light can enter freely into the colloid layer and can act freely on the uniformly distributed sensitive material. For the exposure less light-energy or a shorter duration of exposure is needed, than with the films used hitherto, containing sediments.

Without further analysis, the foregoing will so fully reveal the gist of this invention that others can, by applying current knowledge, readily adapt it for various utilizations by retaining one or more of the features that, from the standpoint of the prior art, fairly constitute essential characteristics of either the generic or specific aspects of this invention and, therefore, such adaptations should be, and are intended to be, comprehended within the meaning and range of equivalency of the following claims.

I claim:—

1. The process of manufacturing photo-sensitive bodies having a colloid layer, which comprises photo-sensitizing said layer with an agent adapted to harden the layer by reaction with light, and treating said bodies with a dilute aqueous solution of an alcohol to free the photo-sensitive surface of non-uniformly distributed sediments, the treatment being continued for only a short time so as to leave the sensitivity of the said bodies substantially unimpaired.

2. The process of manufacturing photo-sensitive bodies having a colloid layer which comprises photo-sensitizing said layer with an agent adapted to harden the layer by reaction with light; and treating said bodies with a dilute aqueous solution of an alcohol immediately after the sensitizing is completed to free the photo-sensitive surface of non-uniformly distributed sediments, the treatment being continued for only a short time so as to leave the sensitivity of the said bodies substantially unimpaired.

3. The process of manufacturing photo-sensitive bodies having a colloid layer which comprises photo-sensitizing said layer with an agent adapted to harden the layer by reaction with light; and treating said bodies with a dilute aqueous solution of an alcohol containing about 10% alcohol to free the photo-sensitive surface of non-uniformly distributed sediments, the treatment being continued for only a short time so as to leave the sensitivity of the said bodies substantially unimpaired.

4. The process of manufacturing photo-sensitive bodies having a colloid layer which comprises photo-sensitizing said layer with an agent adapted to harden the layer by reaction with light; and treating said bodies with a dilute aqueous alcoholic solution which contains about 10% of ethyl alcohol to free the photo-sensitive surface of non-uniformly distributed sediments, the treatment being continued for only a short time so as to leave the sensitivity of the said bodies substantially unimpaired.

5. The process of manufacturing photo-sensitive bodies having a colloid layer which comprises photo-sensitizing said layer with an agent adapted to harden the layer by reaction with light; and treating said bodies for about 10 to 20 seconds with a dilute aqueous solution of an alcohol to free the photo-sensitive surface of non-uniformly distributed sediments, and leaving the sensitivity of said bodies substantially unimpaired.

6. The process of manufacturing photo-sensitive bodies having a colloid layer, which comprises photo-sensitizing said layer with an agent adapted to harden the layer by reaction with light,

immersing said bodies for about 10 to 20 seconds in a bath containing a 10% solution of ethyl alcohol in water immediately after the sensitizing is completed, and subsequently drying said bodies.

7. The process of manufacturing photo-sensitive bodies which comprises coating a suitable carrier with a layer of a colloid, impregnating said layer with a sensitizing liquid containing

chromates and alcohol in aqueous solution; subsequently treating said bodies with a dilute aqueous solution of an alcohol to free the photo-sensitive surface of non-uniformly distributed sediments, the treatment being continued for only a short time so as to leave the sensitivity of the said bodies substantially unimpaired.

CARL ROEHRICH.

85

90

95

100

105

110

115

120

125

130

135

140

145

150

10

15

20

25

30

35

40

45

50

55

60

65

70

75